

Sept. 18, 1973

JOSE MARIA S. AGUIRRE ET AL 3,759,752

PROCESS FOR INCREASING THE MECHANICAL RESISTANCE OF ELEMENTS

MANUFACTURED IN ALLOYS OF LEAD AND ANTIMONY

Filed Aug. 23, 1971

2 Sheets-Sheet 1



Fig. 1

INVENTORS

JOSE MARIA SISTIAGA AGUIRRE  
MARCELINO TORRALBA DIAZ  
JUAN JOSE REGIDOR ARRIBAS  
MIGUEL ABALLE CARIDE

BY

*Richard P. Elkin*

ATTORNEY

Sept. 18, 1973

JOSÉ MARÍA S. AGUIRRE ET AL

3,759,752

PROCESS FOR INCREASING THE MECHANICAL RESISTANCE OF ELEMENTS  
MANUFACTURED IN ALLOYS OF LEAD AND ANTIMONY

Filed Aug. 23, 1971

2 Sheets-Sheet 2



Fig. 2

INVENTORS

JOSE MARIA SISTIAGA AGUIRRE  
MARCELINO TORRALBA DIAZ  
JUAN JOSE REGIDOR ARRIBAS  
MIGUEL ABALLE CARIDE

BY

*Richard P. Elbein*

ATTORNEY

1

3,759,752

PROCESS FOR INCREASING THE MECHANICAL  
RESISTANCE OF ELEMENTS MANUFACTURED  
IN ALLOYS OF LEAD AND ANTIMONY

José-Maria Sistiaga Aguirre, Marcelino Torralba Diaz,  
Juan-José Regidor Arribas, and Miguel Abalie Caride,  
Madrid, Spain, assignors to Patronato de Investigacion  
Cientifica y Tecnica "Juan de la Cierva" del Consejo  
Superior de Investigaciones

Filed Aug. 23, 1971, Ser. No. 174,010

Claims priority, application Spain, June 26, 1971,  
392,689

Int. Cl. C21d 1/62; C22f 1/12  
U.S. Cl. 148—3

2 Claims

#### ABSTRACT OF THE DISCLOSURE

This invention is concerned with alloys of lead and antimony, and more concretely with a thermal treatment that permits the acceleration of the processes of precipitation of antimony which gives rise to the hardening of these alloys, and which consequently permits the obtaining in these alloys of elements of higher mechanical resistance, which makes them more suitable for handling in short periods of time.

#### DESCRIPTION OF PREVIOUS TECHNIQUE

The alloys of lead and antimony can be considered as some of the most widely used in the field of non-ferrous metallurgy due to their use in the manufacture of products whose consumption reaches very important tonnages, such as sheaths for telephone, telegraph and electric power cables, piping, certain elements for the chemical industry, munitions, bearings, printers' metal, screens for protection against penetrating radiation and grids for accumulators. Of all these applications, that which without doubt gives rise to the highest consumption of lead is that mentioned last, for which purpose there are utilised at the present time alloys with contents of 4 to 6 percent of antimony by weight, although some years ago this percentage used to be much higher. The importance of these alloys is made manifest by the fact that in Europe the consumption of lead for this purpose rose between 1963 and 1969 from 314,000 tons to 430,500 tons, and in the same period for time consumption in the United States increased from 398,000 tons to 506,300 tons.

Depending on the end sought, the types of alloys employed can be divided into two main categories: those intended for use in sheaths piping, etc., in which it is endeavoured to increase the mechanical resistance of the lead, maintaining good ductility, use contents of antimony which in general do not exceed 1.25 percent by weight, although they frequently contain other alloying elements. This type of material can be hot-shaped, especially by extrusion.

The other type of alloys is that in which it is desired to have the best possible mechanical resistance without the capacity of the alloys to be shaped being over important, since the pieces are obtained by pouring and do not receive any subsequent mechanical treatment, or at most are subjected to a process of machining. This is the case with grids for accumulators, and with the blocks for constructing protective screens against penetrating radiations, for example. In these cases contents of antimony higher than 4 percent are employed.

The increase of mechanical resistance of these alloys by comparison with pure lead is not due to hardening by solid solution, since antimony alone is soluble in lead at ambient temperature in very small quantities of the order of 0.3 percent. The hardening is produced because, on the material being cooled after manufacture, the anti-

2

mony present precipitates in the form of small particles which distort the network of the lead and make its plastic deformation difficult. When antimony contents higher than 3.5 percent are concerned, during the process of solidification considerable precipitates of antimony are formed which constitute a further contribution to mechanical resistance. It is important to note that the hardening due to precipitation takes some time to be produced, tending towards a maximum value, the lower the temperature the higher the value, but the higher the temperature the sooner this maximum value is produced. After the attainment of this maximum, a new softening is produced. By way of example, an alloy of 2 percent of antimony delays in reaching the maximum hardness, which is approximately 16 HB, some 40 days, after having been made soluble and tempered, when it is kept at 20° C., while the same alloy kept at 80° C. takes only 8 hours to reach the said maximum, but in this case the hardness attained is only 10 HB. For this reason it is necessary to use higher contents of antimony to attain high values of hardness in short periods of time.

In the majority of the applications which we have mentioned as requiring a high mechanical resistance, the product is obtained by molding, a reason for which recourse is also had to high contents of antimony, since the meltability of these alloys is greater the nearer they are to the eutectoid state of 11.1 percent Sb. This problem is not highly critical since it can be resolved by suitably varying the temperature of the molten metal and the mold, a reason for which the content has been reduced to the above-mentioned 4 to 6 percent of antimony.

In some concrete application, such as the manufacture of grids for accumulators, it seems that the presence of antimony gives rise to surfaces that favour the adherence of the active material (paste), but it appears that the adherence is heterogeneous and is related to the heterogeneity of the distribution of the antimony. By way of example of the present situation concerning manufacturing processes, we shall now refer to the case of the manufacture of grids for accumulators. The alloy of lead and antimony with contents that can vary considerably according to the manufacturer, but which generally lie between 4 and 6 percent of antimony, is kept molten at a temperature of some 400 or 450° C. and is poured into a mold of suitable form which is kept at some 180 or 200° C. Once the grid has solidified, it is expelled from the mold and cools rapidly, because of its shape. Under these conditions the cooling of the lead is very rapid, which gives rise to the fact that a considerable part of the antimony is retained in the form of an oversaturated solid solution, the result being that the grid has a mechanical resistance lower than that which it will attain when the whole of the antimony has precipitated. Since the operation of applying paste to the grids requires that the latter have a certain mechanical resistance, since otherwise they would become deformed on paste being applied, producing the consequent paralyzation of the train of the machine, the grids must be kept for a certain time at a suitable temperature so that the antimony will go on precipitating and increasing the hardness. In the treatments of the alloys that are utilised in industry, times are employed which are not sufficiently long, but which cannot be increased, due to economic reasons. Because of this, and since with a lower content of antimony lower values of hardness are attained, for the moment it is difficult to bring about a reduction of the antimony content of these alloys. Nevertheless, this would be desirable, even if only because of the fluctuations of an economic nature that affect the prices of batteries, due to the price of antimony.

Returning to the concrete case of the grids, after they have been stored for a certain time, as has been said, in order to produce hardening through the precipitation of the antimony, they are taken to the pasting machine which carries out the process in a continuous form. The other operations involved in the manufacture of accumulators are well-known, and are not related to the problem being considered here.

Thus, concluding the example, we see that it would be of great interest to achieve the acceleration of the processes of hardening, which would imply a saving in time and, consequently, an economy.

If this is achieved, moreover, for lower contents of antimony, the improvement is even greater. It is also possible to think of the importance that an improvement of this type would have, when it is a question of pieces obtained by molding and which subsequently have to be machined to give them a concrete shape. In such cases the harder the alloy the easier will the machining be, due to the fact that the alloy will be more easily adjustable to the machines used for machining.

#### SUMMARY OF THE INVENTION

The present invention consists of a method of accelerating the processes of aging or precipitation of alloys of lead and antimony, by means of the retention in the network of agents bearing the atoms of antimony, such as are the empty spaces introduced by a rapid cooling, and which on becoming united to the atoms of antimony can produce complexes which are more rapidly diffused through the network. The vacant spaces in the network are physical defects therein which exist in great numbers at high temperatures, but when the material is cooled remain in a metastable equilibrium and consequently tend to become diffused and eliminated. This phenomenon, in the case of alloys of lead and antimony, takes place at high speed at temperatures equal to or greater than the ambient temperature, but nevertheless when the temperature is lowered their mobility diminishes, and consequently they tend to become united to atoms of antimony, thus reducing their metastability and increasing the mobility of the atoms of antimony with which they are associated, which, since they are also initially in a metastable state after cooling, tend to become grouped together, forming precipitates. Again, the lower the temperature at which they are produced the smaller and more abundant are these precipitates, with the result that there is simultaneously attained a finer distribution of the antimony.

Because of this, in order to produce a more rapid aging of the alloy of lead and antimony under consideration, it is sufficient to introduce the piece that it is desired to age more rapidly after it has been cooled, into a bath at a temperature of  $-10^{\circ}$  C. for a time which can vary, according to the alloy, from a few hours to two days, and the longer the duration of the treatment the greater is the effect. The subsequent aging at ambient temperature will take place spectacularly more rapidly, the hardness value after the cold treatment will be significant, and the final precipitation will be finer than if this treatment had not taken place. Again, and since the precipitation is finer, the maximum value of hardness is greater than that presented by the same alloy when it has not undergone the aging treatment in a cool medium. A piece under these conditions can be subjected to machining, or, in the case of an accumulator grid, to the application of paste, more easily than another piece which has not undergone this treatment.

#### DESCRIPTION OF THE PREFERRED VERSION

In its widest aspect, this invention serves to bring about a rapid aging and hardening of pieces of any alloy of lead and antimony. Its preferred version is concerned with the manufacture of grids for accumulators. The modification of the process normally utilised consists in cooling the

grid as rapidly as possible, both when it has been obtained by pouring and when it has been obtained by hot-shaping. Likewise, if the piece has been obtained by cold-shaping, the process can be utilised by previously giving the piece a solution treatment and rapid cooling. In any one of the cases cited, once the piece has been cooled it should immediately be introduced into a bath or a chamber or any other place which is at a temperature below  $20^{\circ}$  C., preferably  $-10^{\circ}$  C. The time that it should remain at this temperature will be established according to the alloy and the degree of hardness it is desired to obtain. Once this time has transpired, the grids are in a condition for paste to be applied to them. In some cases a decision may be taken to maintain the alloy at a low temperature for a shorter period, followed by another period at the ambient temperature prior to the application of the paste.

#### EXAMPLE I

20 A series of wires of some 15 cms. long and 2 mm. in diameter of an alloy Pb-2 percent Sb was taken, and was submitted to a solution treatment at  $240^{\circ}$  C. for 1 hour. The wires were quenched in water at  $10^{\circ}$  C. and immediately afterwards were introduced into a bath of methanol at the temperatures and for the periods indicated in the graph. Subsequently, a study was made of the variation in electrical resistance of these wires, this variation being an index of their state of aging, at the end of four days during which they were kept at ambient temperature. It was seen that the test pieces that had been submitted to a treatment lying between  $0^{\circ}$  C. and  $-10^{\circ}$  C. underwent a much more rapid aging than did the others.

#### Description of the graph of Example I

25 On the graph of FIG. 1 there is represented the value reached by the electrical resistance of test pieces subjected to solution treatments and quenching which have been immediately subjected to the treatments whose times and temperatures are stated on the graph. On the ordinates there is represented the electrical resistance referred to the value it has immediately after the tempering treatment. The abscissa represents the temperature of the sub-ambient treatment in  $^{\circ}$  C.

#### EXAMPLE II

30 Four test pieces of Pb-2 percent Sb were submitted to a solution treatment at  $240^{\circ}$  C. for one hour, and they were then rapidly cooled to  $10^{\circ}$  C. One of the test pieces was left at ambient temperature, and its hardness was checked as time transpired, it being observed, FIG. 2, that it initially had a hardness of 6.0 HB and only at the end of 10 days did it reach a value of 15.0 HB. Another test piece was introduced, immediately after cooling, into a bath at  $-10^{\circ}$  C. and kept there for 3 hours. The effect 35 of this treatment was substantial, since the test piece came to have a hardness of approximately 8.0 HB, and subsequently reached, at ambient temperature, the value of 15.0 HB in only 3 days. Another piece subjected to treatment for 1 day at  $-10^{\circ}$  C. immediately after tempering had, after this treatment, a hardness of 10.5 HB, and at the end of 1 day at ambient temperature had a hardness of 17.0 HB, a value never attained by the test pieces that did not undergo treatment in cold. Finally, when the cold treatment lasts for two days at  $-10^{\circ}$  C., the values are spectacular, since at the end of this treatment the test pieces have a hardness of more than 13.0 HB, and with the passage of time this value rises to nearly 20.0 HB.

#### Description of FIG. 2

40 In the figure there may be seen the evolution of hardness with time in some test pieces of an alloy of Pb-2 percent Sb which have been solution treated and cooled rapidly, and which immediately afterwards have undergone the treatments indicated in FIG. 2.

What is claimed is:

1. A process for increasing the mechanical resistance of elements, comprising the steps of:
  - providing a lead-base alloy comprising 0.3%–11.5% by weight of antimony;
  - heating said alloy to a temperature sufficient to obtain a solid solution of antimony in said lead-base alloy;
  - cooling said alloy rapidly to a temperature of approximately  $-10^{\circ}$  C. and
  - maintaining said alloy at said temperature for a period of from 3 hours to 2 days and thereafter aging the alloy at ambient temperature to achieve the optimum desired hardness.
2. A process for increasing the mechanical resistance of grids for accumulators comprising the steps of:
  - providing a lead-base alloy comprising from between 0.3% to 11.5% by weight of antimony;

melting said alloy;  
 casting said alloy into molds for forming said grids;  
 cooling said alloy rapidly to a temperature of approximately minus  $10^{\circ}$  C.;  
 aging said alloy at said temperature for from 3 hours to 2 days and thereafter aging the alloy at ambient temperature to achieve the optimum desired hardness.

**References Cited**

**UNITED STATES PATENTS**

2,148,741 2/1939 Gonser \_\_\_\_\_ 148—125 X  
 3,008,853 11/1961 Borchers et al. \_\_\_\_ 148—125 X

CHARLES N. LOVELL, Primary Examiner

U.S. CL. X.R.

148—125, 158